

# United States Patent [19]

Turner

[11] 3,862,334

[45] Jan. 21, 1975

[54] **METHOD OF MANUFACTURING CARBON FIBRES** 3,412,062 11/1968 Johnson et al. 23/209.1 X

[75] Inventor: **William N. Turner**, Mickleover, England

*Primary Examiner*—Edward J. Meros  
*Attorney, Agent, or Firm*—Cushman, Darby & Cushman

[73] Assignee: **Secretary of State for Defense**, London, England

[22] Filed: **June 4, 1969**

[21] Appl. No.: **830,534**

## [30] Foreign Application Priority Data

June 4, 1968 Great Britain 26422/68

[52] U.S. Cl. 423/447, 264/29

[51] Int. Cl. C01b 31/07

[58] Field of Search 23/209.1, 209.2, 209.4; 8/115.5, 116; 423/447; 264/29

## [56] References Cited

### UNITED STATES PATENTS

3,285,696 11/1966 Tsunoda 23/209.1

## [57] ABSTRACT

In the manufacture of carbon fibre a process is proposed in which a polymeric fibre is firstly heated to a temperature in the range 200° – 300° C in an inert atmosphere for a predetermined time, secondly heated to a temperature in the range 150° – 250° C in an oxygen containing atmosphere for a predetermined time, and subsequently pyrolysed.

Using this two-stage preoxidation the exothermic nature of the reaction is reduced.

5 Claims, No Drawings

**METHOD OF MANUFACTURING CARBON FIBRES**

This invention relates to a method of manufacturing carbon fibres.

It has previously been proposed to manufacture carbon fibres by the pyrolysis of various starting materials particularly polyacrylonitrile and co-polymers thereof. In this process it has been proposed to use a pre-oxidation step in which the starting fibre is heated in an oxidising atmosphere to a temperature of some 250°C, this pre-oxidation step giving the starting material at least the characteristics of a cross-linked material and hence rendering it more resistant to de-polymerisation so that the subsequent pyrolysis step can be carried out more quickly. One disadvantage of the pre-oxidation treatment as previously proposed lies in its exothermic characteristic which resulted in a considerable output of heat and consequent danger of running away of the reaction and explosion or catastrophic charring of the fibre.

We have invented a method by which the exothermic characteristics of the pre-oxidation may be altered to a far more easily controllable form.

According to the present invention a method of manufacturing carbon fibres comprises the steps of firstly heating a polyacrylonitrile fibre in an inert atmosphere to a temperature in the range 200° to 300°C, secondly heating the fibre in an oxygen containing atmosphere to a temperature in the range 150° to 250°C and subsequently pyrolysing the fibre.

Preferably said pyrolysis step comprises heating the fibre in an inert atmosphere to a temperature in the range 800° to 1,500°C; thus the pyrolysis step may involve heating to 1,000°C in an atmosphere of nitrogen.

The pre-oxidation treatment preferably comprises the first heating step in nitrogen and the second heating step in air, while the first heating step may comprise heating for 3 hours at 210°C, 2 hours at 220°C and 2 hours at 250°C in nitrogen followed by the second step comprising 7 hours at 220°C in air.

The present invention is based on the results of tests we have carried out on the pre-oxidation of, particularly, polyacrylonitrile fibres using a technique known as differential thermal analysis. This technique involves heating the material at a constant rate of temperature rise (6°C per minute) up to about 500°C and accurately measuring the temperature difference between this sample and an inert reference material. Any difference in temperature between the polyacrylonitrile sample and the reference sample indicates either an exotherm or an endotherm depending upon whether the polyacrylonitrile is at a higher or lower temperature than the reference sample.

Carrying out this technique for polyacrylonitrile when heated in air, we found that the reaction showed two exothermic peaks at approximately 250° and 310°C respectively. It will be appreciated that in the prior art pre-oxidation both these exotherms will contribute to the final energy production of the reaction and hence to its likelihood of running away.

Further tests we carried out with the polyacrylonitrile heated in an inert atmosphere showed that the lower temperature exotherm remains even in inert conditions. We believe that the lower temperature exotherm is caused by the conversion of the nitrile group in the original polymer by a cross linking mechanism or alternatively by a ring closure along the polymer molecule chain, while the higher temperature reaction which re-

quires the presence of oxygen results in dehydrogenation and oxygen absorption by the fibre. These reactions are both useful in conferring the necessary stability on the fibre to reduce de-polymerisation and enable a fast heating rate to be used on the subsequent pyrolysis.

This hypothesis was tested by treating fibres first in nitrogen then in air, and it was found by differential thermal analysis that as expected, each treatment produced a single exothermic reaction of less intensity than the combined reaction which occurs merely by heating in air.

It is evident from the above that by heating the fibre first in nitrogen and then in an oxygen containing atmosphere according to the present invention, the two exothermic reactions are separated and thus the stabilisation of the polymer can be achieved with much less danger of running away of the reaction.

In an example of the method according to the invention fibres of a polyacrylonitrile co-polymer known as Courtelle and sold by Messrs Courtaulds Limited were heated in nitrogen for 3 hours at 210°C, 2 hours at 220°C and 2 hours at 250°C. The fibre was subsequently placed in an atmosphere of air and heated at 220°C for 7 hours. The resulting fibre was then pyrolysed by heating to 1,000°C in an inert atmosphere over a time of some 3 hours. The resulting carbon fibre was then tested by standard methods to find the values of Young's modulus and ultimate tensile strength. These values were then compared with values obtained for material which had been pre-oxidised by heating only in air to a temperature of 220°C for some 7 hours then pyrolysed in a nitrogen atmosphere for the same length of time and under the same conditions of temperature as with the fibres pre-treated according to the invention. For the fibres pre-treated according to the invention the mean value of Young's modulus found was  $31 \times 10^6$  psi while the average ultimate tensile strength was  $219 \times 10^3$  psi. These values compared with the values for the fibres not pre-treated according to the invention which gave Young's modulus of  $28 \times 10^6$  psi and an ultimate tensile strength of  $260 \times 10^3$  psi. It will be appreciated that these differences in values are relatively minor and are within the limits of the normal batch-to-batch variations observed using the prior method.

It will be appreciated from these results that the pre-treatment according to the present invention is able to produce fibres of similar strength and modulus to those produced by the prior method while reducing considerably the risk of explosion. In addition we have found that using the two stage pre-treatment of the present invention the temperature of the second step (i.e., heating in an oxygen containing atmosphere) may be effectively carried out at a lower temperature than could be used with the prior art pre-treatment thus allowing further gains in controllability of the pre-treatment and possibly a shortening in overall time.

It will be appreciated that although the invention has been described above with reference to a particular heat treatment, it would be possible to vary the conditions of the heat treatment considerably. Thus we believe that any temperature within the range 200° to 300°C could be used for the first step of heating in an inert atmosphere while any temperature in the range 150° to 250°C is likely to be suitable for a second step of heating in an oxygen containing atmosphere. Of the

various oxygen containing atmospheres which would be useful for the second step, we find air to be the most convenient since its ready availability outweighs any other consideration.

Again although described above with reference to a particular co-polymer of polyacrylonitrile it will be appreciated that the present invention is of use in relation to any polymer to which this combined cross linking and oxygen absorption process is applicable. Obviously this includes other co-polymers of polyacrylonitrile and is in fact also applicable to cellulosic materials such as rayon and polyamide materials such as nylon.

The subsequent pyrolysis of the fibre may be carried out to any temperature in the range 800° to 1,500°C and may also be followed by or include a "graphitisation" treatment which may be performed at any temperature from the pyrolysis temperature up to some 3,500°C depending upon the final properties required of the fibre.

Fibres produced by the method of the present invention may be used in many applications, however, their widest use is as a reinforcing material in a resin matrix, the whole being used as an engineering material for use in such manufactures as gas turbine engines, bearings, etc.

I claim:

1. A method of manufacturing a carbon fibre com-

prising the subsequent steps of firstly heating a polyacrylonitrile fibre in an inert atmosphere to a temperature in the range of 200° to 300°C during which time an exothermic reaction takes place, secondly heating the fibre in an oxygen containing atmosphere to a temperature in the range 150° to 250°C during which time an additional exothermic reaction takes place, and subsequently pyrolysing the fibre.

2. A method as claimed in claim 1 and in which the pyrolysis of the fibre is effected by heating the fibre in an inert atmosphere to a temperature in the range 800° to 1500°C.

3. A method as claimed in claim 2 and in which the pyrolysis of the fibre is effected by heating the fibre to a temperature of about 1,000°C in an atmosphere of nitrogen.

4. A method as claimed in claim 1 in which said first heating step comprises heating the fibre for 3 hours at 210° C, 2 hours at 220° C, and 2 hours at 250° C in an atmosphere of nitrogen, during which time an exothermic reaction takes place.

5. A method as claimed in claim 1 and in which said second heating step comprises heating the fibre in air at a temperature of 220° C for 7 hours during which time an additional exothermic reaction takes place.

\* \* \* \* \*